

Nov. 14, 1961

A. ADAMS ET AL

3,008,655

BENEFICIATION OF POTASH ORES

Filed May 11, 1959



Inventors:

Albert Adams

William B. Dancy

By Ernest V. Haines

Attorney

1

3,008,655

## BENEFICIATION OF POTASH ORES

Albert Adams and William B. Dancy, Carlsbad, N. Mex., assignors to International Minerals & Chemical Corporation, a corporation of New York

Filed May 11, 1959, Ser. No. 812,414

8 Claims. (Cl. 241—20)

The present invention generally relates to the beneficiation of potash ores. More particularly, it relates to an improved process for the recovery of sylvite from ores of the sylvinitite type; for example, such ores as are found in the Permian basin of the southwest area of the United States and mined chiefly in the Carlsbad district of New Mexico, and as are found in the Williston basin of the United States and Canada. The process is, however, applicable to the treatment of other potash ores wherein sylvite is associated with other minerals.

As is well known, potash is of great economic importance. Extensive deposits of potash salts are found on every continent. However, in practically no instance is the potash salt found in a substantially pure form. On the North American continent, one frequently encountered potash salt is sylvite (KCl). The KCl is not often found in any appreciable quantities as pure sylvite, but is most often found as sylvinitite ore, which is a mixture of sylvite and halite (NaCl). A typical analysis of a sylvinitite ore is as follows:

|                                                                               | Percent |
|-------------------------------------------------------------------------------|---------|
| Sylvite (KCl)-----                                                            | 23      |
| Halite (NaCl)-----                                                            | 73      |
| Other constituents or impurities consisting of silicates, sulfates, etc.----- | 4       |

The potash ore in the Williston basin also generally contains carnallite ( $KCl \cdot MgCl_2 \cdot 6H_2O$ ).

Large amounts of sylvite are recovered from sylvinitite ores by processes involving a froth flotation operation. In processes of this general character, it has been the general practice to grind the ore to a rather fine mesh size, for example, to a degree of fineness where at least 90% of the ore would pass through a sieve of about 40 mesh. Flotation of the valuable sylvite constituents from an ore of such a degree of fineness is not too difficult a problem, and various types of collector agents for effecting such flotation can be used.

In a sylvinitite flotation process, the potash ore is slurried in a saturated brine solution to produce a brine slurry or pulp containing from about 50% to about 75% solids. The pulp is reagentized with a suitable collector, diluted with brine, and passed to a flotation cell. In the flotation cell the pulp is kept in circulation and is contacted with air. Air bubbles adhere to the reagentized sylvite particles and float the sylvite particles. The sylvite float is raked off of the top of the flotation cell. Not all of the sylvite is floated off in the first flotation cell and the remaining pulp is removed as underflow from the first cell and is passed to a second flotation cell. In the second cell, the flotation operation is repeated, a sylvite concentrate is floated off, and the remaining pulp may be passed to a third cell. A flotation machine usually contains a plurality, normally five, of such cells associated together in series. After a series of flotation operations, the remaining pulp, from which substantial amounts of sylvite have been removed, is discarded as a tailing. This initial flotation operation is denominated a rougher flotation, the float product is denominated a rougher float or rougher concentrate, and the tailing is denominated a rougher tail.

The rougher concentrate, while containing substantially all of the sylvite values in the charged pulp, also contains a substantial amount of fine halite particles. There-

2

fore, it is conventional practice to combine the rougher concentrate from the individual flotation cells and subject the combined rougher concentrates to a cleaner flotation operation. In the cleaner flotation operation, the rougher concentrate in a pulp is subjected to flotation in another plurality of flotation cells in series. The un floated pulp recovered from the last of the cleaner flotation cells is denominated a middling and is usually recycled to the rougher cells. The float product from the cleaner operation is recovered as a high grade sylvite product, usually denominated a cleaner concentrate.

The flotation of relatively large particles, however, is, in general, attended with considerably more difficulty than when the particles are of relatively smaller size. In other words, it is generally more difficult to float relatively larger size sylvite particles than it is to float relatively smaller size particles. It has been observed that the large sylvite particles make up a substantial amount of the sylvite which is not floated and which is, therefore, usually lost in the tailings.

For many purposes, however, it is undesirable to reduce the mineral to a very small particle size. In the manufacture and utilization of fertilizers, for example, which commonly include phosphate rock and sylvite or other potash mineral, the use of such materials in finely divided form gives rise to caking and dusting problems, so that granular materials are distinctly preferred, and the demand therefor has greatly expanded within recent years. A need has, therefore, existed for a method of beneficiating such minerals in granular form, so that they are directly available to the market without any necessity for separating them first in powdered form and then re converting them into granular form.

Methods have already been devised which achieve flotation of granular materials to some extent. Such methods generally subject an aqueous slurry of the desired material to flotation in the presence of a selective collector reagent such as an amine or a fatty acid, a frothing agent such as an aliphatic alcohol of intermediate molecular weight, and a non-saponifiable oil such as crude petroleum, fuel oil, or kerosene. Recently it has been discovered that the flotation of granular materials is benefited when the flotation mixture contains a viscous petroleum oil having certain characteristics. The viscous petroleum oil preferably has a viscosity at 130° F. greater than about 100 SSU and a distillation range with a 10% point above about 500° F. (ASTM D-447). Many of the so-called "gas oils," lubricating oil stocks, and paraffin or wax distillates obtained in the distillation of crude oils and in the redistillation of cracked stocks and heavy distillates have been found suitable.

It has been found by extensive study that the flotation of sylvite, especially granular sylvite, is markedly inhibited by the presence of slime-forming clay compounds. The term "slimes," as used herein, includes very fine particles, such as clays. The term "slimes" is well known to those skilled in the art of beneficiating potash ores and it is used herein as it is conventionally used in the art.

The slimes associated with potash ores are, however, very difficult to remove. The present invention is concerned with the problem of providing a low slime content feed to a flotation operation.

Accordingly, it is an object of the present invention to provide a process for beneficiating potash ore.

It is another object of the invention to provide a process for preparing a low slime content potash feed material.

It is a further object to provide a flotation process for the flotation of granular sylvite from sylvinitite type ores.

It is an additional object to provide an improved process for the recovery of sylvite from sylvinitic ores, which process includes a flotation operation and a desliming step.

These and other objects and advantages of the present invention will be apparent to those skilled in the art as the description of the present invention progresses.

In accordance with the present invention, it has been discovered that eminently satisfactory beneficiation of potash ores and minerals can be achieved by means of a series of critical and interdependent process steps.

Generally described, the present invention is a process for beneficiating a potash ore which comprises subjecting a comminuted potash ore containing sylvite to a sizing treatment to provide at least two fractions, a first finer fraction composed principally of finer particles of said ore and a first coarser fraction comprised principally of coarser particles of said ore, separately comminuting the first coarser fraction, subjecting the comminuted coarser fraction to a sizing treatment to provide at least two fractions, a second finer fraction composed principally of finer particles of the comminuted first coarser fraction and a second coarser fraction composed principally of coarser particles of the comminuted first coarser fraction, combining at least a portion of the first finer fraction with at least a portion of the second finer fraction, separately conditioning at least a portion of the second coarser fraction with cationic collecting agent and then subjecting the combined finer fraction and the conditioned second coarser fraction to froth flotation concentration.

In order to more fully appreciate the present invention with its many advantages, reference may be made to the accompanying drawing which is a diagrammatic flow-sheet illustrating the general application of the process of the invention.

In this novel process, potash ore containing sylvite, for example, sylvinitic ore as received from the mine, is comminuted to economical liberation size to produce a granular feed material. The ore is comminuted, usually dry crushed, to reduce substantially all of the ore to less than about  $\frac{3}{8}$  inch size. During the crushing to  $\frac{3}{8}$  inch, a substantial portion of the ore is reduced to  $-20$  mesh. It has been determined that the  $-20$  mesh material contains the major portion of the liberated slimes, for example, 70% of the slimes in the ore, and, in accordance with the present invention, the comminuted ore is subjected to a sizing treatment to provide at least two fractions, a first finer fraction composed principally of finer particles of the comminuted ore and a first coarser fraction composed principally of coarser particles of the ore. The comminuted ore is preferably sized on about 20 mesh so that the fine fraction is predominantly  $-20$  mesh and the coarse fraction  $+20$  mesh. As hereinabove set forth, it has been determined that the  $-20$  mesh material contains the major portion of the liberated slimes in the ore. Since the presence of slimes is particularly harmful in the flotation of granular sylvite, the materials in the first finer fraction are never again admixed with materials in the first coarser fraction until these materials are first conditioned for flotation. In other words, the first coarser fraction is treated in its own circuit, which usually is called the granular circuit, including the step of conditioning, and the first finer fraction is also separately treated in its own circuit, which usually is called the fines circuit, including the step of conditioning. After conditioning, the conditioned materials in the main processing streams may be admixed and then subjected to flotation or, alternately, the conditioned materials may be separately subjected to flotation. Further, when in any subsequent operation on the first coarser fraction, a relatively smaller size fraction is produced, for example, in a hydrocycloning and/or classification of the material in the first coarser fraction, it is preferable that such smaller size fraction be removed

from contact with the coarser fraction until the coarser fraction is conditioned for flotation. These embodiments are illustrated in the accompanying drawing.

The comminuted ore from the crusher is slurried with a brine solution which is substantially saturated with respect to sylvite and also substantially saturated with respect to halite, and is then introduced into a classifier, termed the primary classifier, for the first sizing operation. For the sake of simplicity, and in order to present the invention in a clearer manner, the sizing in the primary classifier will be considered to be on 20 mesh. Sizing on 20 mesh is preferred since a beneficial split of slimes and sylvite is achieved on this size; however, it will be apparent to those skilled in the art that another mesh size may be used and it is, therefore, to be understood that the sizing may be on another predetermined mesh size. Also, in the subsequent description, which may very readily be followed by referring to the drawing, certain mesh sizes are specified. These specified mesh sizes are also preferred; however, it will again be apparent to those skilled in the art that another mesh size may be used with equivalent results and it is, therefore, to be understood that the sizing may be on other predetermined mesh sizes. The other mesh sizes will preferably be close to the mesh sizes specified in the description.

In the classifier, the operating conditions are maintained so as to obtain a pulp overflow composed principally of  $-20$  mesh particles. This  $-20$  mesh fraction is treated in its own fine circuit which is illustrated in the drawing chiefly in the left half of the drawing. The underflow from the classifier is composed principally of  $+20$  mesh particles and is treated in its own granular circuit which is illustrated in the drawing chiefly in the right half of the drawing.

Directing attention first to the treatment of the  $+20$  mesh fraction, this fraction also contains a substantial portion of  $+8$  mesh material which is too large for efficient flotation. The  $+20$  mesh fraction is accordingly introduced into a so-called slime mill for wet grinding to reduce the coarser particles to a suitable size for a flotation feed. The wet grinding is preferably done in a rod mill since it has been determined that in a rod mill, very fine particles are not produced in too great an amount. The wet grinding operation is regulated so that the out flow from the rod mill is predominantly  $-8$   $+20$  mesh material. In general, it has been determined that the degree of size reduction depends, to some extent, upon one or more of the following: pulp density of the feed material, relationship between the volume of grinding media and the volume of the mill, the rod charge, the diameter of the rods, and the speed of the mill.

The discharge from the slime mill is introduced into a hydrocyclone, termed the granular hydrocyclone, for the removal of fines and liberated slimes produced in the slime mill. One or a bank of hydrocyclones in parallel may, of course, be used. The material is fed tangentially into the hydrocyclone. In the hydrocyclone a separation is made in the cone-shaped part by the action of centrifugal and centripetal forces. A discussion of hydrocyclones of this type may be found in Perry, Chemical Engineer's Handbook, third edition. The cones are selected and operated to effect a separation on about 35 mesh. The  $-35$  mesh material is removed as overflow from the hydrocyclone. This  $-35$  mesh material usually contains a significant amount of slimes and is, therefore, in accordance with the invention, removed from the granular circuit. Accordingly, the  $-35$  mesh material is removed from the granular circuit and is introduced with the  $-20$  mesh overflow from the primary classifier into a primary hydroseparator in the fines circuit.

The  $+35$  mesh underflow from the granular hydrocyclone is introduced into a secondary classifier for another sizing operation. In this secondary classifier, the operating conditions are maintained so as to obtain a

pulp overflow composed principally of -20 mesh particles and a pulp underflow composed principally of +20 mesh particles. Looking back at the operation of the granular cyclone, it should be noted that -35 mesh material is taken off as overflow, and in the secondary classifier -20 mesh material is taken off as overflow. Such an operation is preferred since it has been determined that improved results are obtained when treating the -35 mesh fraction and the -20 mesh fraction separately in the fines treating circuit. The further treatment accorded each of these fractions will be described in detail hereinafter. It should, however, be noted at this time that the material in the -20 mesh overflow from the secondary classifier does not come into contact with any of the material in the granular circuit before the granular material is conditioned for flotation.

The -20 mesh overflow from the secondary classifier usually still contains some -200 mesh ore and slime particles. The -20 mesh material is, therefore, subjected to a sizing in a secondary hydrocyclone on about 48 mesh. The -48 mesh overflow fraction from the secondary hydrocyclone is introduced into a second hydroseparater in the fines circuit hereinafter described in detail. The +48 mesh hydrocyclone underflow fraction contains predominantly -20 +48 mesh particles. The +48 mesh fraction is substantially free of slimes and is passed to a fines conditioner for suitable conditioning for flotation.

The +20 mesh slurry underflow from the secondary classifier is introduced into a granular conditioner wherein the material is treated with flotation reagents. For proper conditioning the material is preferably in the form of a relatively thick pulp, usually from about 50% to about 75% solid content, and when necessary, brine may be added to the +20 mesh underflow. In the granular conditioner, the material is preferably conditioned with a cationic collector, a slime controllant and a viscous petroleum oil. A frothing agent may also be added. These materials are conventionally employed in the flotation of sylvite and they are employed in conventional manner and amounts.

The cationic collector includes aliphatic amines such as n-lauryl amine. Other useful collector agents are high molecular weight aliphatic amines of about C-14 to C-20 length carbon chains and their water-soluble acid addition salts, as well as quaternary ammonium salts, preferably the acetate or hydrochlorides, for example, octadecylamine acetate, hexadecylamine hydrochloride, and the like. High molecular weight aliphatic amines and their water-soluble acetate salts are commercially available. The collector floats potassium chloride particles.

The slime controllant is also used in conventional manner and in conventional amount. Various slime control agents are known and starch is preferred. Other slime control agents are the polyglycol and polyglycol ethers disclosed in U.S. Patent No. 2,724,499. Other slime control agents are sold by Dow Chemical Company and General Mills, Incorporated.

The viscous petroleum oil is also employed in conventional manner and in conventional amounts, generally between about 0.5 and about 5.0 pounds per ton of solids. It has been determined that a more selective and more complete flotation of the granular sylvite from the granular ore mixture is achieved by the use of the viscous petroleum oil. The oil preferably has a pour-point of 50° F. to 100° F., a viscosity above about 100 S.S.U. at 130° F. and below 300 S.S.U., preferably above about 150 S.S.U. and should be largely a high-boiling point material, having a distillation temperature (ASTM D-447) above about 500° F. at the 10% distillation level. A further description of suitable oils may be found in Trachta and Rodriguez co-pending patent application Serial No. 781,462, filed December 19, 1958.

It is also conventional to incorporate in the flotation mixture a suitable frothing agent, such as an aliphatic

alcohol of intermediate molecular weight (around C<sub>4</sub>-C<sub>10</sub>), a preferred example being methyl isobutyl carbinol. Other frothing agents are described in the art.

After conditioning, the slurry is diluted with brine to the desired degree for froth flotation, preferably to a solids concentration between about 20% and about 35% solids, and subjected to a froth flotation operation.

The fines circuit starts at the overflow from the primary classifier. The -20 mesh fraction overflowing from the primary classifier is introduced into a primary hydroseparater. The -35 mesh overflow from the granular hydrocyclone is also introduced into this primary hydroseparater. The primary hydroseparater is of a suitable type for slime removal. The rates of feed and agitation, as well as other operating variables, are so regulated during the desliming step as to insure an overflow which contains predominantly -200 mesh particles of the ore and the liberated insoluble slimes. In general, -200 mesh sylvite particles are too small to be efficiently beneficiated

in a froth flotation operation. The -200 mesh fraction is usually sent to brine clarification thickeners wherein the solids are permitted to settle out so that the clarified brine may be reused.

The +200 mesh underflow fraction from the primary hydroseparater is then passed to a fines hydrocyclone for a sizing operation. In general, the +200 mesh material still contains a considerable amount of liberated slimes and -200 mesh material. The fines hydrocyclone is selected and operated to effect a sizing on about 48 mesh.

A hydrocyclone usually operates more efficiently at a solids content less than is present in the +200 mesh underflow fraction and, therefore, brine is usually added to dilute the +200 mesh fraction to the desired degree for hydrocycloning.

The +48 mesh underflow fraction from the fines hydrocyclone is sufficiently free of slimes to be amenable to conditioning and froth flotation. This material is accordingly passed, with other materials, into the fines conditioner.

The -48 mesh overflow fraction from the fines hydrocyclone and the -48 mesh overflow from the secondary hydrocyclone are passed into a second hydroseparater. In this second hydroseparater, as in the primary hydroseparater, the rates of feed, agitation, and other operating conditions are regulated so as to achieve desliming or sizing at about 200 mesh. The -200 mesh overflow from the second hydroseparater is sent to brine clarification. The +200 mesh underflow is substantially free of slimes and other -200 mesh material and is introduced into the fines conditioner.

In the fines conditioner, the material is treated with a slime controllant in conventional manner and in conventional amount. Starch is a preferred slime controllant; however, other materials, for example the materials discussed as slime control agents for the granular conditioning, may be used. When the conditioned fines material is combined with the condition granular material for flotation, a cationic agent need not be added to the fines conditioner.

However, when the fines conditioned material is separately treated in its own fine fraction flotation circuit, a cationic flotation reagent is also added to the conditioner. In general, the cationic agents suitable for such use are the same as those described for use in the granular conditioner.

The aliphatic amines for the fine conditioning may be of relatively lower molecular weight as compared to the aliphatic amines used in the granular conditioning.

In a commercial operation, when the operation was changed from a conventional feed preparation process to the process of the present invention, the production of -8 +20 mesh granular sylvite increased 40%.

The following examples are given to illustrate the instant novel process and are not to be construed as limiting the invention thereto.

7  
EXAMPLE I

This example illustrates a specific commercial application of the invention.

A sylvinite ore as received from the mine had the following analysis:

## Mineral analysis

|                           | Percent |
|---------------------------|---------|
| Clay                      | 1.0     |
| Sylvite                   | 22.0    |
| Halite and other minerals | 77.0    |

This ore was crushed to substantially all  $-\frac{3}{8}$  inch size. 400 tons per hour of the crushed ore was slurried with a saturated brine solution to 42% solids and introduced into a primary classifier. The classifier was operated so as to produce about 100 tons per hour of  $-20$  mesh overflow (24% solids) and about 300 tons per hour of  $+20$  mesh sands or underflow (70% solids). The  $+20$  mesh sands or underflow was introduced into a rod mill wherein the charge was comminuted to produce a predominantly  $-8$   $+20$  mesh fraction. The discharge from the rod mill was introduced into a granular hydrocyclone.

The granular hydrocyclone provided 5.0 tons per hour of a  $-35$  mesh overflow (16% solids) and 225 tons per hour of a  $+35$  mesh underflow. The  $+35$  mesh underflow was introduced into a secondary classifier. The secondary classifier was operated to produce a substantially  $-20$  mesh overflow at the rate of 55 tons per hour (8% solids) and a substantially  $+20$  mesh sands or underflow at the rate of 170 tons per hour (70% solids). The  $+20$  mesh fraction was passed to a granular conditioner and conditioned at 60% solids. This  $+20$  mesh fraction contained only 0.08% slimes. Potato starch was added to the solids in the conditioner at the rate of 0.3 pound per ton of solids. An amine flotation reagent, comprising a mixture of Armee TD, n-octadecylamine, and Armee HTD, sold by Armour and Company, was then added to the conditioner at the rate of 2.20 pounds per ton of feed. A highly paraffinic, viscous, fractionator bottoms material produced at the Malco Oil Co. refinery at Artesia, New Mexico, was also introduced into the conditioner at the rate of 0.72 pound per ton of feed.

The  $-20$  mesh overflow from the secondary classifier was passed to a secondary hydrocyclone which was operated to size at about 48 mesh. The  $-48$  mesh overflow (3% solids) was removed at the rate of 215 tons per hour. The  $+48$  mesh underflow (70% solids) was 21 tons per hour. The  $+48$  mesh fraction contained only 0.08% slimes and was sent to the fines conditioner.

Referring back to the primary classifier, the  $-20$  mesh overflow was introduced into a primary hydroseparatory along with the  $-35$  mesh overflow from the granular hydrocyclone. The primary hydroseparatory was operated to produce a  $-200$  mesh overflow (1.6% solids) at 510 tons per hour. The  $+200$  mesh underflow (47% solids) at 180 tons per hour was diluted with fresh brine to 40% solids and then passed into a fines hydrocyclone.

The fines hydrocyclone was operated to size at about 48 mesh. The  $+48$  mesh underflow (68% solids) at 53 tons per hour contained only 0.11% slimes, and was passed directly to the fines conditioner. The  $-48$  mesh overflow (22% solids) at 170 tons per hour from the fines hydrocyclone was introduced into a second hydroseparatory along with the  $-48$  mesh overflow from the secondary hydrocyclone.

The second hydroseparatory was operated to remove a  $-200$  mesh overflow (1.2% solids) at 330 tons per hour and a  $+200$  mesh underflow (48% solids) at 110 tons per hour. The  $+200$  mesh underflow was passed to the fines conditioner.

Three main processing streams are, accordingly, being passed into the fines conditioner. From the second hydroseparatory 52 tons per hour of  $+200$  mesh material, from the secondary hydrocyclone 49 tons per hour of

8  
+48 mesh material, and from the fines hydrocyclone 110 tons per hour of  $+48$  mesh material.

In the fines conditioner the material was conditioned with potato starch, which was added to give 1.1 lbs. of starch per ton of solids.

The conditioned fines material at 211 tons per hour was combined with the conditioned granular material at 170 tons per hour and the combined stream (381 tons per hour) was diluted with fresh brine to 28% solids and then passed through a conventional rougher and cleaner flotation process. The sylvite product had a 61.6%  $K_2O$  content and had the following analysis:

TABLE I

| $K_2O$ Analysis | Mesh Size Analysis |
|-----------------|--------------------|
| 62.5%           | $-8+20, 26.0\%$    |
| 61.3%           | $-20+65, 55.0\%$   |
| 60.2%           | $-65, 19.0\%$      |

## EXAMPLE II

A sylvinite ore as received from the mine had the following analysis:

## Mineral analysis

|                           | Percent |
|---------------------------|---------|
| Clay                      | 1.0     |
| Sylvite                   | 22.0    |
| Halite and other minerals | 77.0    |

The ore was crushed to substantially all  $-\frac{3}{8}$  inch size. 400 tons per hour of the crushed ore was slurried with a saturated brine solution to 42% solids and introduced into a primary classifier. The classifier was operated to size on about 20 mesh with 100 ton per hour of  $-20$  mesh overflow (24% solids) and 300 tons per hour of  $+20$  mesh underflow (70% solids). The  $+20$  mesh fraction was comminuted in a rod mill to substantially all  $-8$  mesh material.

## Operation A

In one operation, designated operation A, the rod mill discharge was recombined with the  $-20$  mesh overflow from the primary classifier and the combined stream was then washed and classified on 20 mesh to produce a substantially  $-20$  mesh fraction and a substantially  $+20$  mesh fraction. The  $+20$  mesh fraction was passed to a conditioner and conditioned at 60% solids with potato starch, amine, and the highly paraffinic, viscous, fractionator bottom material, in substantially the same manner and amounts as the  $+20$  mesh fraction described in Example I was conditioned. The  $-20$  mesh fraction was deslimed by washing and then separately conditioned with 1.1 lbs. of potato starch per ton of solids. The conditioned fractions were then combined and subjected to conventional froth flotation to produce a sylvite concentrate.

## Operation B

In another operation, designated operation B, which operation is in accordance with the process of this invention, the rod mill discharge was subjected to washing and classification on 20 mesh with the  $-20$  mesh fraction from this classification being combined with  $-20$  mesh overflow from the primary classifier. The combined  $-20$  mesh fraction was deslimed by washing and then conditioned with potato starch in substantially the same manner as the  $-20$  mesh fraction in operation A. The  $+20$  mesh fraction was also conditioned in substantially the same manner as the  $+20$  mesh fraction in operation A. The conditioned fractions were then combined and subjected to conventional froth flotation to produce a sylvite concentrate.

Comparing operations A and B, it may be noted that the primary difference in the processes is that in operation A, the rod mill discharge is combined with the primary classifier overflow and the combined stream is then classi-

fied to produce the -20 mesh fraction and the +20 mesh fraction which are separately subjected to conditioning prior to flotation, while in operation B, the rod mill discharge is not first combined with the primary classifier overflow, but the rod mill discharge is classified to provide the +20 mesh fraction which is separately conditioned and a -20 mesh fraction which is combined with the primary classifier overflow to provide the -20 mesh fraction which is separately conditioned.

The sylvite products from operations A and B were collected and analyzed. The results of the analysis and a comparison of operations are shown below in Table 2.

TABLE 2

| Screen Analysis Mesh Size             | Operation A | Operation B |
|---------------------------------------|-------------|-------------|
| +10                                   | nil         | 0.9         |
| +14                                   | 1.5         | 7.3         |
| +20                                   | 5.4         | 21.6        |
| Percent Recovery of Coarser Fraction: |             |             |
| +10                                   | 24          | 55          |
| -10 +14                               | 51          | 82          |
| -14 +20                               | 84          | 94          |
| K <sub>2</sub> O Analysis of Product  | 60.85       | 61.15       |

From Table 2, it may be seen that when following operation B, which is in accordance with the present invention, more +20 material was in the product and, further, the overall K<sub>2</sub>O content of the product was higher.

The description of the invention utilized specific reference to certain process details; however, it is to be understood that such details are illustrative only and not by way of limitation. Other modifications and equivalents of the invention will be apparent to those skilled in the art from the foregoing description.

Having now fully described and illustrated the invention, what is desired to be secured and claimed by Letters Patent is set forth in the appended claims:

1. A process for beneficiating a potash ore which comprises subjecting a comminuted potash ore containing sylvite to a sizing treatment to provide at least two fractions, a first finer fraction composed principally of finer particles of said ore and a first coarser fraction composed principally of coarser particles of said ore, separately comminuting the first coarser fraction, separately subjecting the comminuted coarser fraction to a sizing treatment to provide at least two fractions, a second finer fraction composed principally of finer particles of the comminuted first coarser fraction and a second coarser fraction composed principally of coarser particles of the comminuted first coarser fraction, combining at least a portion of the first finer fraction with at least a portion of the second finer fraction, conditioning the combined finer fraction with a slime controllant, separately conditioning at least a portion of the second coarser fraction with a cationic collecting agent and then subjecting the conditioned combined finer fraction and the conditioned second coarser fraction to froth flotation concentration.

2. A process for beneficiating a potash ore which comprises comminuting a potash ore containing sylvite to reduce substantially all of the ore to less than about  $\frac{3}{8}$  inch size, subjecting the comminuted potash ore to a sizing treatment to provide at least two fractions, a first finer fraction composed principally of -20 mesh particles of said ore and a first coarser fraction composed principally of +20 mesh particles of said ore, separately comminuting the first coarser fraction, separately subjecting the comminuted coarser fraction to a sizing treatment to provide at least two fractions, a second finer fraction composed principally of finer particles of the comminuted first coarser fraction and a second coarser fraction composed principally of coarser particles of the comminuted first coarser fraction, combining at least a portion of the first finer fraction with at least a portion of the second finer fraction, conditioning the combined finer fraction with a slime controllant, separately conditioning at least a portion of the second coarser fraction with a cationic collecting agent, combining at least a portion of the conditioned combined finer fraction with at least a portion of the conditioned second coarser fraction, and then subjecting the combined fractions to froth flotation concentration.

3. A process for beneficiating a potash ore which comprises comminuting a potash ore containing sylvite to reduce substantially all of the ore to less than about  $\frac{3}{8}$  inch size, subjecting the comminuted potash ore to a sizing treatment to provide at least two fractions, a first

10 finer fraction composed principally of -20 mesh particles of said ore and a first coarser fraction composed principally of +20 mesh particles of said ore, separately comminuting the first coarser fraction to substantially all -8 mesh size particles, separately subjecting the comminuted coarser fraction to a sizing treatment to provide at least two fractions, a second finer fraction composed principally of -20 mesh particles of the comminuted first coarser fraction and a second coarser fraction composed principally of +20 mesh particles of the comminuted first coarser fraction, combining at least a portion of the first finer fraction with at least a portion of the second finer fraction, conditioning the combined finer fraction with a slime controllant, separately conditioning at least a portion of the second coarser fraction with a cationic collecting agent and then subjecting the conditioned combined finer fraction and the conditioned second coarser fraction to froth flotation concentration.

4. A process for beneficiating a potash ore which comprises subjecting a comminuted potash ore containing sylvite to a sizing treatment to provide at least two fractions, a first finer fraction composed principally of finer particles of said ore and a first coarser fraction composed principally of coarser particles of said ore, separately comminuting the first coarser fraction, separately subjecting the comminuted coarser fraction to a sizing treatment to provide at least two fractions, a second finer fraction composed principally of finer particles of the comminuted first coarser fraction and a second coarser fraction composed principally of coarser particles of the comminuted first coarser fraction, combining at least a portion of the first finer fraction with at least a portion of the second finer fraction, separately conditioning at least a portion of the second coarser fraction with a cationic collecting agent and subjecting the conditioned combined finer fraction to froth flotation concentration.

5. A process for beneficiating a potash ore which comprises subjecting a comminuted potash ore containing sylvite to a sizing treatment to provide at least two fractions, a first finer fraction composed principally of finer particles of said ore and a first coarser fraction composed principally of coarser particles of said ore, separately comminuting the first coarser fraction, separately subjecting the comminuted coarser fraction to a sizing treatment to provide at least two fractions, a second finer fraction composed principally of finer particles of the comminuted first coarser fraction and a second coarser

60 fraction composed principally of coarser particles of the comminuted first coarser fraction, combining at least a portion of the first finer fraction with at least a portion of the second finer fraction, conditioning the combined finer fraction with a slime controllant, separately conditioning at least a portion of the second coarser fraction with a cationic collecting agent, combining at least a portion of the conditioned combined finer fraction with at least a portion of the conditioned second coarser fraction, and then subjecting the combined fractions to froth flotation concentration.

6. A process for beneficiating a potash ore which comprises subjecting a comminuted potash ore containing sylvite to a sizing treatment to provide at least two fractions, a first finer fraction composed principally of finer

particles of said ore and a first coarser fraction composed principally of coarser particles of said ore, separately comminuting the first coarser fraction, separately subjecting the comminuted coarser fraction to a sizing treatment to provide at least two fractions, a second finer fraction composed principally of finer particles of the comminuted first coarser fraction and a second coarser fraction composed principally of coarser particles of the comminuted first coarser fraction, combining at least a portion of the first finer fraction with at least a portion of the second finer fraction, separately conditioning at least a portion of the second coarser fraction with a cationic collecting agent and separately conditioning at least a portion of the finer fraction with starch, combining at least a portion of the starch conditioned combined finer fraction with at least a portion of the conditioned second coarser fraction, and then subjecting the combined coarser and finer fraction to froth flotation concentration, and recovering a sylvite concentrate.

7. A process for beneficiating a potash ore which comprises comminuting a potash ore containing sylvite to reduce substantially all of the ore to less than about  $\frac{3}{8}$  inch size, subjecting the comminuted potash ore to a sizing treatment to provide at least two fractions, a first finer fraction composed principally of -20 mesh particles of said ore and a first coarser fraction composed principally of +20 mesh particles of said ore, separately comminuting the first coarser fraction, separately subjecting the comminuted coarser fraction to a sizing treatment to provide at least two fractions, a second finer fraction composed principally of finer particles of the comminuted first coarser fraction and a second coarser fraction composed principally of coarser particles of the comminuted first coarser fraction, combining at least a portion of the first finer fraction with at least a portion of the second finer fraction, separately conditioning at least a portion of the second coarser fraction with a cationic collecting agent and separately conditioning at least a portion

of the finer fraction with starch, combining at least a portion of the starch conditioned combined finer fraction with at least a portion of the conditioned second coarser fraction, and then subjecting the combined coarser and finer fraction to froth flotation concentration, and recovering a sylvite concentrate.

8. A process for beneficiating a potash ore which comprises comminuting a potash ore containing sylvite to reduce substantially all of the ore to less than about  $\frac{3}{8}$  inch size, subjecting the comminuted potash ore to a sizing treatment to provide at least two fractions, a first finer fraction composed principally of -20 mesh particles of said ore and a first coarser fraction composed principally of +20 mesh particles of said ore, separately 10 comminuting the first coarser fraction to substantially all -8 mesh size particles, separately subjecting the comminuted coarser fraction to a sizing treatment to provide at least two fractions, a second finer fraction composed principally of -20 mesh particles of the comminuted 15 first coarser fraction and a second coarser fraction composed principally of +20 mesh particles of the comminuted first coarser fraction, combining at least a portion of the comminuted first coarser fraction, combining at least a portion of the first finer fraction with at least a fraction of the second finer portion, separately conditioning at least 20 a portion of the second coarser fraction with an amine collecting agent and separately conditioning at least a portion of the finer fraction with starch, combining at least a portion of the starch conditioned combined finer fraction with at least a portion of the conditioned second 25 coarser fraction, and then subjecting the combined coarser and finer fraction to froth flotation concentration and recovering a sylvite concentrate.

## References Cited in the file of this patent

## UNITED STATES PATENTS

- |           |                    |              |
|-----------|--------------------|--------------|
| 2,836,297 | Smith et al. ----- | May 27, 1958 |
| 2,846,068 | Smith et al. ----- | Aug. 5, 1958 |